

1,296,035.

A. B. ANDREWS.

METHOD OF EXTRACTING POTASH AND THE LIKE,  
APPLICATION FILED MAR. 6, 1918.

Patented Mar. 4, 1919.



Inventor,  
Arthur B. Andrews  
by *Alis S. Scott*  
attorney

# UNITED STATES PATENT OFFICE.

ARTHUR BURTON ANDREWS, OF AUBURN, MAINE, ASSIGNOR OF ONE-HALF TO HIMSELF AND ONE-HALF TO HERBERT F. KELLEY, OF AUBURN, MAINE.

## METHOD OF EXTRACTING POTASH AND THE LIKE.

1,296,035.

Specification of Letters Patent.

Patented Mar. 4, 1919.

Application filed March 6, 1918. Serial No. 220,824.

*To all whom it may concern:*

Be it known that I, ARTHUR B. ANDREWS, a citizen of the United States, residing at Auburn, county of Androscoggin, State of Maine, have invented certain new and useful Improvements in Methods of Extracting Potash and the like, of which the following is a specification.

This invention relates to the extraction of the alkaline content from silicates, especially such as feldspar, and particularly to the recovery of potassium in the form of potassium hydroxid by which a yield is secured with a maximum of recovery of the potassium content, and with a minimum difficulty as to those incidents of extraction which have been such serious factors in effecting a rapid and efficient production.

My method is based on the old and well known digestion of feldspar with lime. In extraction by this process as in almost all other digestive processes, the two incidents of the process which make for expense in operation and limitation of output are the elements of time and pressure. Each of these factors as is obvious constitutes features of serious cost in production. It is perfectly obvious that the time consumed in the process of digestion is a factor in both expense and quantity in output, and in the same manner the higher the degree of pressure used, the greater the expense of equipment and the higher the cost of operation.

It is therefore obviously very highly desirable to devise a method in which these two incidents of time and pressure be minimized as far as possible. It is probably sufficient to note that there has been considerable misapprehension as to the relation of these two collateral features of the digestive process.

It has been supposed by some that sustained cooking or increase of pressure or both would increase yield, while some have set up some definite time or pressure as controlling the entire problem. I have found, however, that sustained cooking and increased pressure may easily be carried to a point where the process begins to reverse and rebuild the silicates. I also find that

the time and the degree of pressure varies 50 with different feldspars and must be determined by experiment for the individual circumstances of different feldspars and different methods. As will be more clearly pointed out later on, both of these items are 55 incident to the rates of digestive reaction, the completeness and rapidity and economy of the reaction being the important element of the method, and constituting the thing desired, while the time or pressure are incidental factors to be reduced as low as possible by the efficiency of the method.

My method consists, broadly speaking, of increasing the rapidity and completeness of the reaction by dividing the ordinary digestive method into steps in accordance with principles which will be hereinafter explained, so that a maximum extraction of the caustic is effected with a minimum of material and at a substantial saving of time 70 and pressure.

I have discovered that the rate of reaction in the digestive process between feldspar and the lime has a certain maximum phase bearing relation to the strength of 75 the caustic solution as it is in contact. In other words, the reaction proceeds more rapidly and more easily (thus involving less heat and pressure) up to a certain per cent. of caustic strength of solution, after which 80 the rate of reaction falls off rapidly, eventually reaching a point at which the reaction begins to reverse so that it is actually possible by digesting too long and at too high pressure to again break up the caustic and 85 begin to reform it as a silicate.

My method therefore contemplates a division of the digestion into a fractional series and an opposite progression in the fractional digestions so that the liquor of maximum strength is brought into digestive relation with the material of minimum potential reaction and vice versa. This fractional digestion in such a series increases the net rate of reaction at a considerable 90 saving of time and will do so at comparatively low pressures. It furthermore by reason of its augmentive action builds up a

liquor of maximum strength and effects an extraction of from 95% to 98% of the alkali content.

Any suitable apparatus may be employed 5 in my invention such as digesters, presses, suitable tanks, pumps and piping, all as is well known in the art and all arranged most conveniently according to the available space of the particular plant in which the method 10 is to be practised, so that no illustration thereof is necessary. I preferably employ three digesters, although two or even more than three may be employed, as conditions require. Feldspar and caustic lime are introduced 15 into a digester at one end of the series and to it is added the liquor from the next preceding digester, which liquor is we will say nearly completed and which has a minimum of reactive tendency and thus requires 20 the maximum tendency of the fresh charge in order to raise its strength.

The digester from which this liquor comes is fed with the sludge from the first-named digester which in the triple battery for example, would be the first digester. In this second or middle digester therefore, I combine the sludge consisting of the partly decomposed and extracted material from the first digester with the weak liquor from the 25 third digester. This weak liquor has still a considerable reactive potentiality which can be largely satisfied by even the partially extracted sludge from the first mentioned digester. The sludge from this second mentioned or middle digestor is fed over to a digester in which it is mixed with fresh water and to which is added such wash water as is obtained in the final washing of any previous sludge after it has had its third 30 reaction and before it is dumped out as the reject. This reject has had taken from it, according somewhat to the character of the materials used 95% to 98% of its alkaline content.

45 Tracing the course of the liquor through the system it will be found (on the basis of a 10%  $K_2O$  feldspar) that the water which has been digested with the sludge of two previous extractions will frequently be found to constitute 50 a liquor of as high as one-half per cent. strength caustic potash. This liquor after digestion with the once digested sludge in the middle digester will be found to be augmented usually to about nine-tenths per cent. strength caustic potash, and the ultimate liquor from the digestion with the fresh material will be found to have a strength of about one and three-tenths per cent., which may then be economically 55 evaporated in a multiple effect evaporator, and finally dried in a fusion pan and packaged for shipment. The charge of each digester after cooking is separated by suitable filterings and washings into a sludge 60 and a liquor.

For convenience in visualizing my method, I have illustrated in the single figure of the annexed drawing a graph descriptive of my method.

Various modifications may obviously be 70 practised in the method and the results may vary somewhat with the efficiency of the apparatus and the skill and care employed in its operation. It may be stated, however, that I have been able to produce by my 75 method as high as 98% extraction of potash from feldspar of about 10%  $K_2O$  at average runs of six hours and employing only pressures of 75 and 100 pounds. The amount of lime required for ordinary operations is 80 preferably of amount approximately double in weight to the amount of the feldspar. I also preferably supply the feldspar in very finely divided condition.

What I therefore claim and desire to secure by Letters Patent is:

1. The process of extracting alkali from silicates consisting in a progressive fractional digestion with an alkaline earth metal hydrate by separating the liquor and sludge 90 of each fractional digestion and adding the liquor of the most digested sludge to a less digested sludge.

2. The process of extracting alkali from silicates consisting in a series of progressive fractional digestions with an alkaline earth metal hydrate by establishing from successive digestions of successive charges a series of liquors of increasing strength and in successively digesting each digested 100 charge with the liquor of the preceding digestion in the series.

3. The process of extracting alkali from silicates by digestion with an alkaline earth metal hydrate consisting in establishing a 105 fractional digestive series in which the silicate and hydrate is introduced at the finishing end of the liquor and water is introduced at the opposite end of the series, the liquor from the water end being progressed to digestive contact with each sludge and each sludge being progressed for said digestive contact with each liquor.

4. The process of extracting alkali from silicates by digestion with an alkaline earth 110 metal hydrate consisting in establishing a series of simultaneous fractional digestions and in maintaining said fractional digestions by adding the augmented liquor of one digestion to the sludge from which the next 120 stronger batch of liquor was augmented.

5. The process of extracting alkali from silicates by digestion with an alkaline earth metal hydrate consisting in establishing a series of simultaneous fractional digestions 125 and in maintaining said fractional digestions by adding the augmented liquor of one digestion to the sludge from which the next stronger batch of liquor was augmented, and in evaporating the ultimate liquor so found. 130

6. The process of making caustic potash from feldspar by digestion with lime consisting in digestively treating each successive charge of feldspar and lime with the  
5 liquor of a digestive treatment of the sludge of the preceding charge.

In testimony whereof I affix my signature in presence of two witnesses.

ARTHUR BURTON ANDREWS.

Witnesses:

EDITH M. DUNN,  
CHAS. B. CARTER.

Copies of this patent may be obtained for five cents each, by addressing the "Commissioner of Patents, Washington, D. C."